

July 29, 1924.

1,502,983

P. A. DIEFENTHÄLER

PRODUCTION OF GRAY CAST IRON

Filed April 2, 1921



Philip August Diefenthaler

INVENTOR

BY *W. J. B. Whitney*

ATTORNEY

Patented July 29, 1924.

1,502,983

# UNITED STATES PATENT OFFICE.

PHILIPP AUGUST DIEFENTHÄLER, OF HEIDELBERG, GERMANY, ASSIGNOR TO THE FIRM HEINRICH LANZ, OF MANNHEIM, BADEN, GERMANY, A COPARTNERSHIP.

## PRODUCTION OF GRAY CAST IRON.

Application filed April 2, 1921. Serial No. 458,049.

(GRANTED UNDER THE PROVISIONS OF THE ACT OF MARCH 3, 1921, 41 STAT. L., 1313.)

*To all whom it may concern:*

Be it known that I, PHILIPP AUGUST DIEFENTHÄLER, residing at 5<sup>a</sup> Rombachweg, Heidelberg, Baden, Germany, have invented **5** certain new and useful Improvements in and Relating to the Production of Gray Cast Iron (for which I filed applications in Germany, D32,571, May 9, 1916, Pat. No. 301,913; Austria, A6118/18, Nov. 23, 1918, **10** Pat. No. 80,884; Hungary, D3,121, Nov. 6, 1918, Pat. No. 75,662), of which the following is a specification.

In the use of cast iron for machine parts, which are subjected to much friction, such as **15** bearings, steam cylinders, slide blocks, pistons, guides, and the like, for a long time, conflicting and very often unsatisfactory results have been experienced. Whilst in some cases, such articles last well in use for **20** many years, other machine parts of the same kind soon wear away and, by running hot and corroding, often lead to difficulties in operation. It has been attempted to overcome these drawbacks by producing the cast iron exactly on the basis of analytical experiments without, however, leading to uniform results.

I have discovered that it is absolutely necessary to produce a definite texture or structural condition in such articles in order, in **30** all circumstances, to exclude the difficulties referred to.

The congealing diagram of cast iron shows, as is well known, two distinct conditions: on the one hand, iron with combined carbon, and on the other hand iron with the carbon in the form of graphite. Between these two limiting conditions—cementite on the one side and ferrite on the other side—**35** the transitional condition of pearlite is formed. I have found that a well-developed, uniformly distributed, lamellar pearlite structure, with moderate graphite veining, no free ferrite being formed, gives the **40** casting, besides great strength, the capacity of withstanding frictional wear to a very great degree.

Such a structure is illustrated in the accompanying drawing, wherein is shown a **50** microphotograph of a somewhat large complex, magnified 250 times, composed of several granules of banded pearlite with only interspersed veinings *a* of graphite.

The invention consists, therefore, in producing the casting according to the rules of **55** the iron-carbon crystallization doctrine and conducting its cooling in such a way that in the finished piece of work the lamellar pearlite form predominates. This object is obtained advantageously by a cast iron composition, with a low content of carbon, silicon, manganese, phosphorus and sulphur. The essentials of the process are, firstly, a suitable cast iron composition and, secondly, **60** cooling gradually in the mould so as to obtain the desired structure in the casting. The thickness of the casting, and other factors on which the cooling rate depends, must be taken into account and in order to obtain **65** with certainty the lamellar pearlite structure, excluding free ferrite, desired, the cooling should be effected as gradually as possible.

The solution of the problem, therefore, **70** consists in first choosing such a composition of low carbon and silicon content as to allow the forming of pearlite and graphite and finding out empirically, for a definite composition and the different cross-sections of the casting, the heat curve according to **75** which with certainty the desired pearlite structure is obtained and then cooling the finished casting in the mould according to this temperature curve. This can be done, **80** for example, satisfactorily by bringing the mould preliminarily to a definite temperature. It has been found, for example, in the case of a composition of 3 per cent carbon (of which 0.85 per cent is combined with **85** the iron and thus forms pearlite and the remaining 2.15 per cent occurs as finely distributed graphite), 1 per cent silicon, 0.7 per cent manganese, 0.4 per cent phosphorus, 0.1 per cent sulphur and 94.8 per cent iron that the mould should be preliminarily **90** heated to the following temperatures:

For a thickness of material of about 10 millimeters to about 390° F.

For a thickness of material of about 20 millimeters to about 300° F. **100**

For a thickness of material of about 30 millimetres to about 210° F.

If the composition is different, for example, if it contains only about 2.8 per cent carbon (of which 0.85 per cent is combined **105** with the iron and 1.95 per cent occurs as fine-

ly distributed graphite) and 0.8 per cent silicon, the preliminary temperature of the mould should be selected about 70° to 80° F. higher, that is to say:—

5 For a thickness of 10 millimetres about 470° F.

For a thickness of 20 millimetres about 380° F.

10 For a thickness of 30 millimetres about 290° F.

It may be seen from these examples, that it is a comparatively simple matter to prepare scales or curves for a particular composition from which, without further trouble, the necessary temperature of the mould can be read for a particular thickness of material.

20 Alternative methods of carrying out the process to produce the lamellar pearlite structure consist in heating the molten iron to a higher temperature such that the excess of heat serves for the necessary heating of the mould or by inserting the mould after casting in a heated chamber the temperature of which can be easily regulated so as to cool the casting according to the empirically obtained cooling conditions.

30 For preheating the mould a heated chamber may be employed through which the mould is drawn by means of a transporter band or similar means, the duration of travel and temperature of chamber being such that the mould acquires the requisite temperature. The same chamber can be used for the latter of the two alternative methods mentioned. Accordingly the metal is cast in a cold mould and the mould is brought into the heated chamber as quickly as possible and left therein for a sufficient 40 time to permit the pearlite structure to develop. In this case also empirical curves can be readily plotted from which according to the composition, the thickness of the casting and the temperature prevailing in the chamber the requisite duration of the passage of the mould through the chamber can be read off. When the mould is taken out of the chamber it is allowed to cool in the ordinary way.

45 50 According to these technical rules, it is possible to produce gray cast iron which will stand frictional wear to a very high degree.

55 What I claim as new, and desire to secure by Letters Patent, is—

1. The method of producing gray cast iron having a uniformly distributed lamellar pearlite structure with moderate veinings of graphite and with little if any free ferrite which consists in making the castings from an iron composition with a low content of carbon and silicon and in heating the mould to a temperature above normal to artificially retard the cooling of the castings therein and permit the pearlite structure to develop. 60

2. The method of producing gray cast iron of predominantly lamellar pearlite structure and of high resistivity to frictional wear which consists in using for the castings an iron composition having a low content of carbon, silicon, manganese, phosphorous and sulphur and in retarding the cooling of the castings in the mould according to temperature curves, based upon 70 the heating of the mould to a temperature varying according to the particular composition and the thickness of the casting, adapted to limit the formation both of free ferrite and of cementite. 75

3. The method of producing gray cast iron of predominantly lamellar pearlite structure which comprises starting with an iron composition having a low content of carbon and of silicon and retarding the cooling of the castings, as by cooling them in moulds heated above normal to a temperature dependent upon the particular composition used and the thickness of the castings, to the extent required for the development of 80 the pearlite structure. 85

4. Gray cast iron of great strength and highly resistant to frictional wear which throughout is composed predominantly of well-developed and uniformly distributed 95 lamellar pearlite.

5. Gray cast iron which is characterized by a uniform pearlite structure with interposed strata of finely distributed graphite and with little if any free ferrite. 100

6. Gray cast iron having a well-developed and uniformly distributed lamellar pearlite structure with moderate graphite veinings and with little if any free ferrite.

In testimony whereof I have affixed my 105 signature in presence of two witnesses.

PHILIPP AUGUST DIEFENTHÄLER.

Witnesses:

MAX STRAUSS,  
ERIC LEHMANN.

110